



U.S. PATENT DOCUMENTS

|                 |         |                        |         |
|-----------------|---------|------------------------|---------|
| 4,947,927 A *   | 8/1990  | Horton .....           | 164/517 |
| 4,966,225 A     | 10/1990 | Johnson                |         |
| 4,996,175 A     | 2/1991  | Sturgis                |         |
| 4,998,581 A *   | 3/1991  | Lane et al. .....      | 164/517 |
| 5,299,619 A     | 4/1994  | Chandley et al.        |         |
| 5,407,001 A     | 4/1995  | Yasrebi et al.         |         |
| 5,464,797 A     | 11/1995 | Yasrebi et al.         |         |
| 5,492,957 A *   | 2/1996  | Nishikawa et al. ..... | 524/430 |
| 5,997,802 A     | 12/1999 | Holcombe, Jr. et al.   |         |
| 6,024,163 A     | 2/2000  | Springgate et al.      |         |
| 6,352,101 B1 *  | 3/2002  | Ghosh et al. .....     | 164/516 |
| 2004/0191546 A1 | 9/2004  | Takai et al.           |         |

|    |              |         |
|----|--------------|---------|
| JP | 01184392 A   | 7/1989  |
| JP | 03282187 A   | 12/1991 |
| JP | 2001208481 A | 8/2001  |
| JP | 2003056988 A | 2/2003  |
| WO | 2007039310 A | 4/2007  |

OTHER PUBLICATIONS

|                                                                          |
|--------------------------------------------------------------------------|
| EP 08154904.0, European Search Report and Written Opinion, Jul. 9, 2008. |
| EP 08154903.2, European Search Report and Written Opinion, Jul. 4, 2008. |

FOREIGN PATENT DOCUMENTS

|    |            |        |
|----|------------|--------|
| GB | 569852 A   | 6/1945 |
| JP | 01139988 A | 6/1989 |

\* cited by examiner



FIG. 1



FIG. 2



FIG. 3



FIG. 4





FIG. 6



FIG. 7



FIG. 8

## 1

**METHODS FOR MAKING REINFORCED  
REFRACTORY CRUCIBLES FOR MELTING  
TITANIUM ALLOYS**

**CROSS REFERENCE TO RELATED  
APPLICATIONS**

This application claims priority to U.S. Provisional Application Ser. No. 60/914,935, filed Apr. 30, 2007, which is herein incorporated by reference in its entirety.

**TECHNICAL FIELD**

Embodiments described herein generally relate to methods for making reinforced crucibles suitable for melting titanium alloys. More particularly, embodiments herein generally describe methods for making reinforced refractory crucibles suitable for melting highly reactive titanium alloys, such as titanium aluminide.

**BACKGROUND OF THE INVENTION**

Turbine engine designers are continuously looking for new materials with improved properties for reducing engine weight and obtaining higher engine operating temperatures. Titanium alloys, and in particular, titanium aluminide (TiAl) based alloys, possess a promising combination of low-temperature mechanical properties, such as room temperature ductility and toughness, as well as high intermediate temperature strength and creep resistance. For these reasons, TiAl-based alloys have the potential to replace nickel-based superalloys, which are currently used to make numerous turbine engine components.

Vacuum induction melting is one method often used to make turbine engine components, such as airfoils, and generally involves heating a metal in a crucible made from a non-conductive refractory alloy oxide until the charge of metal within the crucible is melted down to liquid form. When melting highly reactive metals such as titanium or titanium alloys, vacuum induction melting using cold wall or graphite crucibles is typically employed. This is because melting and casting from ceramic crucibles can introduce significant thermal stress on the crucible, which can result in the crucible cracking. Such cracking can reduce crucible life and cause inclusions in the component being cast.

Moreover, difficulties can arise when melting highly reactive alloys, such as TiAl, due to the reactivity of the elements in the alloy at the temperatures needed for melting to occur. As previously mentioned, while most vacuum induction melting systems use refractory alloy oxides for crucibles in the induction furnace, alloys such as TiAl are so highly reactive that they can attack the refractory alloys present in the crucible and contaminate the titanium alloy. For example, ceramic crucibles are typically avoided because the highly reactive TiAl alloys can break down the crucible and contaminate the titanium alloy with both oxygen and the refractory alloy from the oxide. Similarly, if graphite crucibles are employed, the titanium aluminide can dissolve large quantities of carbon from the crucible into the titanium alloy, thereby resulting in contamination. Such contamination results in the loss of mechanical properties of the titanium alloy.

Additionally, while cold crucible melting can offer metallurgical advantages for the processing of the highly reactive alloys described previously, it also has a number of technical and economic limitations including low superheat, yield

## 2

losses due to skull formation and high power requirements. These limitations can restrict commercial viability.

Accordingly, there remains a need for methods for making reinforced crucibles for use in melting highly reactive alloys that are more resistant to thermal stresses generated during the casting process and less likely to contaminate the alloy.

**BRIEF DESCRIPTION OF THE INVENTION**

10 Embodiments herein generally relate to methods for making reinforced refractory crucibles for melting titanium alloys comprising providing a form; applying a facecoat to the form, the facecoat having at least one facecoat layer; applying a backing about the facecoat, the backing having at least one 15 backing layer; applying at least one reinforcing element to at least a portion of the facecoat layer, the backing layer, or a combination thereof wherein the reinforcing element comprises at least one composition selected from the group 20 consisting of ceramic compositions, metallic compositions, and combinations thereof.

Embodiments herein also generally relate to methods for making reinforced refractory crucibles for melting titanium alloys comprising providing a form; applying a facecoat to the form, the facecoat having at least one facecoat layer; 25 applying a backing about the facecoat, the backing having at least one backing layer; applying at least one reinforcing element to at least a portion of the facecoat layer, the backing layer, or a combination thereof wherein the reinforcing element comprises a configuration selected from the group consisting of a continuous fiber, a tape, a mesh, a chopped fiber, and combinations thereof.

Embodiments herein also generally relate to methods for making reinforced refractory crucibles for melting titanium alloys comprising providing a form; applying a facecoat to the form, the facecoat having at least one facecoat layer; applying a backing about the facecoat to produce a crucible mold, the backing having at least one backing layer; applying a stucco layer to each of the at least one facecoat layer and the 35 at least one backing layer; applying a reinforcing element to at least a portion of the facecoat layer, the backing layer, the stucco layer, or a combination thereof wherein the reinforcing element comprises a composition selected from the group consisting of ceramic compositions, metallic compositions, and combinations thereof, removing the form from the crucible mold; and firing the crucible mold to produce the reinforced crucible for melting titanium alloys wherein the reinforcing element comprises a configuration selected from the group consisting of a continuous fiber, a tape, a mesh, a 40 chopped fiber, and combinations thereof and wherein the reinforcing element is tailored to support particular stresses 45 present in different regions of the crucible.

These and other features, aspects and advantages will become evident to those skilled in the art from the following disclosure.

**BRIEF DESCRIPTION OF THE DRAWINGS**

While the specification concludes with claims particularly pointing out and distinctly claiming the invention, it is believed that the embodiments set forth herein will be better understood from the following description in conjunction with the accompanying figures, in which like reference numerals identify like elements.

FIG. 1 is a schematic perspective view of one embodiment of a crucible in accordance with the description herein;

FIG. 2 is a schematic perspective view of one embodiment of a form in accordance with the description herein;

FIG. 3 is a schematic cross-sectional view of one embodiment of a crucible mold in accordance with the description herein;

FIG. 4 is a schematic close-up view of a portion of a cross-section of the crucible mold of FIG. 3;

FIG. 5 is an elevated front view of one embodiment of a crucible mold with reinforcing elements positioned in an adjacent orientation in accordance with the description herein;

FIG. 6 is an elevated front view of one embodiment of a crucible mold with two reinforcing elements, each applied to a different layer of the crucible mold, in accordance with the description herein;

FIG. 7 is an elevated front view of one embodiment of a crucible mold with reinforcing elements positioned in a stacked orientation in accordance with the description herein; and

FIG. 8 is a schematic cross-sectional view of one embodiment of a crucible mold after the form has been removed and a topcoat applied in accordance with the description herein.

#### DETAILED DESCRIPTION OF THE INVENTION

Embodiments described herein generally relate to methods for making refractory crucibles suitable for melting titanium alloys. More specifically, embodiments described herein generally relate to methods for making reinforced refractory crucibles for melting titanium alloys comprising providing a form; applying a facecoat to the form, the facecoat having at least one facecoat layer; applying a backing about the facecoat, the backing having at least one backing layer; applying at least one reinforcing element to at least a portion of the facecoat layer, the backing layer, or a combination thereof wherein the reinforcing element comprises at least one composition selected from the group consisting of ceramic compositions, metallic compositions, and combinations thereof.

While embodiments herein will generally focus on methods for making reinforced crucibles suitable for melting TiAl for use in making near net shape airfoils, the description should not be limited to such. Those skilled in the art will understand that the present embodiments may be used to make reinforced crucibles suitable for melting any titanium alloy for use in making any near net shape gas turbine component.

Turning to FIG. 1, embodiments herein relate to a refractory crucible 8 suitable for melting titanium alloys. Crucible 8 can have an interior 9 and can be made in accordance with the description herein below. To begin, a crucible mold can be made. As used herein “mold” refers to the unfired components that when fired under suitable conditions form crucible 8 of FIG. 1. To make a crucible mold, a form 10 can be provided, as shown in FIG. 2. While form 10 can comprise any material capable of removal from the crucible mold, in one embodiment, form 10 can comprise wax, plastic or wood, and may be hollow or solid. Moreover, form 10 can take any shape and have any dimension necessary to produce the desired interior of the crucible and may comprise a handle 12, or other like mechanism, for ease of handling.

As shown in FIGS. 3 and 4, a facecoat 16 comprising at least one facecoat layer 18, and optionally at least one stucco layer 20, can be applied to form 10. As used herein throughout, “at least one” means that there may be one or more than one and specific layers will be designated herein throughout as “first facecoat layer,” “second facecoat layer,” and the like. Since facecoat layer 18 can be exposed to the TiAl during the melting process, facecoat layer 18 should be inert to the reactive TiAl so as not to degrade and contaminate the alloy

during melting. Therefore, in one embodiment, face coat layer 18 may comprise an oxide. As used herein throughout, “oxide” refers to a composition selected from the group consisting of scandium oxide, yttrium oxide, hafnium oxide, a lanthanide series oxide, and combinations thereof. Furthermore, the lanthanide series oxide (also known as “rare earth” compositions) may comprise an oxide selected from the group consisting of lanthanum oxide, cerium oxide, praseodymium oxide, neodymium oxide, promethium oxide, 10 samarium oxide, europium oxide, gadolinium oxide, terbium oxide, dysprosium oxide, holmium oxide, erbium oxide, ytterbium oxide, lutetium oxide, and combinations thereof.

Facecoat layer 18 may comprise a facecoat slurry made from a powder of the oxide mixed into a colloidal suspension. 15 In one embodiment, the oxide powder may be a small particle powder having a size of less than about 70 microns, and in another embodiment, from about 0.001 microns to about 50 microns, and in yet another embodiment from about 1 micron to about 50 microns. The colloid can be any colloid that gels 20 in a controlled fashion and is inert to TiAl, such as, for example, colloidal silica, colloidal yttria, colloidal alumina, colloidal calcium oxide, colloidal magnesium oxide, colloidal zirconium dioxide, colloidal lanthanide series oxides, and mixtures thereof. While any of the previously listed oxides 25 can be used to make the facecoat slurry of facecoat layer 18, in one embodiment, the facecoat slurry may comprise yttrium oxide particles in a colloidal silica suspension, while in another embodiment, the facecoat slurry may comprise yttrium oxide particles in a colloidal yttria suspension. The 30 composition of the facecoat slurry can vary, however, in general, the facecoat slurry may comprise from about 40% to about 100% of the oxide and from about 0% to about 60% of the colloid, by weight.

Once the facecoat slurry of facecoat layer 18 is prepared 35 using conventional practices, form 10 may be exposed to the facecoat slurry using a method selected from the group consisting of dipping, spraying, and combinations thereof. Generally, once applied, facecoat layer 18 can have a thickness of from about 50 microns to about 500 microns, and in one 40 embodiment from about 150 microns to about 300 microns, and in yet another embodiment about 200 microns.

While still wet, facecoat layer 18 may optionally be coated 45 with a stucco layer 20, as shown in FIGS. 3 and 4. As used herein, “stucco” refers to coarse ceramic particles generally having a size greater than about 100 microns, and in one embodiment from about 100 microns to about 5000 microns. Stucco 20 can be applied to each facecoat layer to help build 50 up the thickness of the crucible wall and provide additional strength. A variety of materials may be suitable for use as stucco layer 20, however, in one embodiment, the stucco may comprise a refractory material, such as, but not limited to, alumina or aluminosilicates, combined with an oxide, as defined herein. The ratio of the refractory material to the oxide in stucco layer 20 can vary, however, in one embodiment, stucco layer 20 can comprise from about 0% to about 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 94

stucco layers 20, are present, though those skilled in the art will understand that facecoat 16 may comprise any number of facecoat layers and stucco layers. While each facecoat layer 18 may comprise a different oxide/colloid mixture, in one embodiment, each facecoat layer 18 comprises the same oxide/colloid mixture. Once the desired number of facecoat layers 18 and stucco layers 20 have been applied, a backing 22 may then be applied.

Backing 22 can help provide additional strength and durability to the finished crucible 8. As such, backing 22 may consist of at least one backing layer 24, shown in FIG. 4, which can comprise a backing slurry including a refractory material selected from the group consisting of aluminum oxide, zirconium silicate, silicon dioxide, and combinations thereof, in a colloidal silica suspension. Specific layers may be designated herein throughout as "first backing layer," "second backing layer," and the like. As an example, in one embodiment, backing layer 24 may comprise a backing slurry made from aluminum oxide particles in a colloidal silica suspension. The composition of the backing slurry can vary, however, in general, the backing slurry may comprise from about 10% to about 40% of the refractory material and from about 60% to about 90% of the colloid, both by weight. Similar to the facecoat layers, each backing layer 24 may optionally comprise a stucco layer 20 adhered thereto, as shown in FIG. 4, which may be the same as or different from the stucco used previously to make the facecoat. Each backing layer 24, including the stucco, can have a thickness of from about 150 microns to about 4000 microns, and in one embodiment from about 150 microns to about 1500 microns, and in yet another embodiment about 700 microns.

Similar to the facecoat layers, each backing layer 24 may be applied using a method selected from the group consisting of dipping, spraying, and combinations thereof. While any number of backing layers 24 can be applied, in one embodiment, there may be from 2 to 40 backing layers. Each backing layer 24 may comprise the same composition of refractory material and colloid, each may be different, or they may comprise some combination in between. After applying the desired number of backing layers, and optional stucco layers, the resulting crucible mold 26 can be further processed.

It should be noted that in some cases it may be desirable to grade the stucco layers by altering particle size, layer thickness and/or composition as they are applied. As used herein, the term "grade," and all forms thereof, refers to gradually increasing the strength of subsequently applied stucco layers by, for example, increasing the particle size of the stucco material, increasing the thickness of the stucco layer and/or utilizing increasingly stronger refractory material/colloid compositions as the stucco layer. Such grading can allow the stucco layers to be tailored to account for differences in thermal expansion and chemical properties of the various facecoat layers and backing layers to which they are applied. More specifically, grading the stucco layers provides differing porosities and can adjust the modulus of the crucible, which taken together, can help account for the differences in thermal expansion as previously discussed.

At any time during the construction of the crucible mold, at least one reinforcing element 14 may be applied to at least a portion of any one or more of facecoat layer 18, backing layer 24, or a stucco layer 20 thereof. In the embodiments of FIGS. 3, 4, 5 and 8, reinforcing element 14 is shown applied to a stucco layer 20 of facecoat 16. However, those skilled in the art will understand that this embodiment is for illustration purposes only and should not be used to limit the scope of the present description.

Reinforcing element may comprise anything capable of increasing the strength of the finished crucible and its resistance to thermal cracking in comparison to crucibles lacking such reinforcing elements. As used herein, "reinforcing element" refers to compositions applied to one or more layers of the crucible mold during construction, rather than to oxides, refractory materials and/or colloids present in the layers of the crucible mold that may react to form reinforcing materials during the firing of the crucible mold, as explained herein.

10 While reinforcing element 14 may be made from any number of compositions, in one embodiment, reinforcing element 14 may comprise a composition selected from the group consisting of ceramic compositions, metallic compositions and combinations thereof. More specifically, reinforcing element 14 may comprise at least one ceramic composition selected from the group consisting of yttria, alumina, sapphire, nitride, yttrium aluminum garnet (YAG), silicon carbide (SiC), silicon aluminum oxinitride (such as SiAlON<sup>TM</sup>), silica, mullite (such as NEXTEL<sup>TM</sup>), zirconia, zircon, zircar, 15 and combinations thereof; at least one metallic composition selected from the group consisting of tungsten, tantalum, molybdenum, niobium, rhenium, alloys thereof, and combinations thereof. Additionally, reinforcing element 14 may comprise a combination of ceramic compositions and metallic compositions, known as cermets, which can include, but should not be limited to, alumina-50% molybdenum, alumina-90% molybdenum, alumina-50% tungsten, and alumina-90% tungsten, by volume.

Reinforcing element 14 may comprise any configuration 30 capable of providing increased strength and resistance to thermal cracking to the finished crucible. In one embodiment, reinforcing element 14 may comprise a configuration selected from the group consisting of a continuous fiber, tape, mesh, chopped fiber, and combinations thereof. The dimensions of the configuration may vary, such as by width, thickness, weave, and the like, according to characteristics desired in the reinforcing element. However, in one embodiment, reinforcing element can have a thickness of less than about 2000 microns, and in another embodiment from about 100 35 microns to about 1000 microns.

40 Additionally, a single configuration may be applied, or more than one configuration may be applied, to the same layer, or different layers, of the crucible mold. If more than one reinforcing element is applied to the same layer, the 45 reinforcing elements may be applied in an adjacent orientation, a stacked orientation, or some combination thereof, as described herein below. For instance, in one embodiment shown in FIG. 5, both a continuous fiber element and a mesh element may be applied to the same layer in an adjacent orientation. In another embodiment shown in FIG. 6, a mesh element and chopped fiber elements may be applied to different layers. In yet another embodiment shown in FIG. 7, a tape element and chopped fiber elements may be applied to the same layer in a stacked orientation.

50 Moreover, reinforcing element 14, the composition thereof, and the configuration thereof, may be selected to support particular stresses present in different regions of the crucible, such as the base region 30, the transition region 32 (i.e. the portion connecting base region 30 to lower region 34), the lower region 34 (i.e. the sides containing the titanium melt during casting), the upper region 36 (i.e. the sides above the titanium melt during casting) 34, and the pour lip region 38, as indicated generally in FIG. 5. In particular, as bending 55 stresses may be significant in base 30, transition 32, and pour lip 36 regions, it may be desirable to utilize at least a mesh reinforcing element 14 in these regions, as shown in FIG. 5. Similarly, in the sides of the crucible (i.e. the upper 36 and

lower 34 regions), hoop stresses will generally be the principal concern and thus, it may be desirable to utilize at least a continuous fiber reinforcing element 14 in such regions, as shown in FIG. 5. By specifically tailoring the reinforcing element to the particular regions of the crucible, thermal stress resistance can be optimized to help ensure the crucible maintains its integrity throughout the heating, melting, pouring, and cool-down phases.

Regardless of the composition or configuration of reinforcing element 14, the application thereof generally follows the same procedure. The at least one reinforcing element 14 may be applied about the selected layer, or layers, while the slurry is still wet. Applying reinforcing element 14 while the selected layer is still wet allows reinforcing element 14 to become secured to crucible mold 26. More particularly, as the selected layer of crucible mold 26 dries, reinforcing element 14 can adhere thereto. The application of reinforcing element 14 can include, but should not be limited to, wrapping or winding reinforcing element 14 about the selected layer(s) of crucible mold 26, as shown in FIGS. 5 and 7, or in the case of chopped fibers, pressing or dusting reinforcing element 14 in the desired location or locations about the selected layer of crucible mold 26, as shown in FIGS. 6 and 7. If more than one reinforcing element is used, and a stacked orientation is selected (see FIG. 7 for example), the previously described techniques can be employed to apply one reinforcing element over another. Those skilled in the art will understand that the reinforcing elements can be either selectively placed about at least a portion of a selected layer of the crucible mold, or alternately, about and entire selected layer of the crucible mold.

Crucible mold 26 may then be dried using conventional practices and form 10 may be removed. A variety of methods may be used to remove form 10 from crucible mold 26. As previously mentioned, form 10 may comprise wax and therefore may be removed by placing crucible mold 26 in a furnace, steam autoclave, microwave, or other like device, and melting form 10 leaving an open interior 9 in crucible mold 26, as shown in FIG. 8. The temperature required to melt form 10 from crucible mold 26 can generally be low and in one embodiment, can range from about 40° C. to about 120° C.

Optionally, interior 9 of crucible mold 26 may then be washed with a colloidal slurry to form a topcoat 28, as shown in FIG. 8. Washing can generally involve applying a coating to the interior of the crucible using any method known to those skilled in the art, such as spraying, prior to firing the crucible. Topcoat 28 can have any desired thickness, however, in one embodiment, topcoat 28 has a thickness of up to about 500 microns, and in another embodiment from about 20 microns to about 400 microns. Topcoat 28 can comprise a colloidal slurry selected from the group consisting of yttria in a colloidal yttria suspension, yttria in a colloidal silica suspension, and combinations thereof. This topcoat can help further ensure that the crucible will remain inert with respect to the titanium alloy during melting.

The hollow crucible mold 26 can then be fired to higher temperatures. Firing crucible mold 26 can help provide additional strength to the finished crucible because during this heating process, the materials that make up the facecoat layers, stucco, and backing layers can interdiffuse with one another and sinter together. Initially, the crucible mold can be fired to a temperature of from about 800° C. to about 1400° C., and in one embodiment from about 900° C. to about 1100° C., and in one embodiment about 1000° C. This first firing can take place for any length of time needed to help burn off any remaining form material, as well as provide a limited degree of interdiffusion among the ceramic constituents of the cru-

cible, which in one embodiment may be from about 0.5 hours to about 50 hours, in another embodiment from about 1 hour to about 30 hours, and in yet another embodiment about 2 hours. Next, the crucible mold can be fired to a temperature of from about 1400° C. to about 1800° C., and in one embodiment from about 1500° C. to about 1800° C., and in yet another embodiment from about 1600° C. to about 1700° C. This second firing can take place for any length of time needed to substantially complete the interdiffusion of the ceramic constituents, as well as cause a reaction of the colloid present in the facecoat oxide, which in one embodiment may be from about 0.5 hours to about 50 hours, in another embodiment from about 1 hour to about 30 hours, and in yet another embodiment about 2 hours. For example, colloidal silica can form silicates, while colloidal yttria can sinter with yttria particles present in the slurry of the facecoat.

Once firing is complete, the resulting crucible can be suitable for use in melting titanium alloys. While specific characteristics of crucible 8 can be altered or modified depending on the desired use, in one embodiment, crucible 8 can have an overall wall thickness, that includes all facecoat layers, stucco layers and backing layers, of at least about 3 mm, and in another embodiment at least about 6 mm, and in yet another embodiment from about 6.5 mm to about 40 mm. Wall thicknesses of greater than about 40 mm can lead to undesirably long high heating times. Similarly, the thickness ratio of the backing to the facecoat can, in one embodiment, be from about 6.5:1 to about 20:1. As above, thickness ratios greater than about 20:1 can result in undesirably long high heating times due to the thickness of the alumina backing layers.

Regardless of the specific construction, crucible 8 may be used to melt titanium alloys having a low interstitial level and a low ceramic inclusion content. In particular, TiAl can be melted in the crucible described herein using conventional melting and casting techniques known to those skilled in the art. The crucibles described herein are capable of use with such highly reactive alloys because the materials used to make the facecoat are inert to the reactive TiAl. In other words, the facecoat can be exposed to the TiAl during melting without degrading and contaminating the alloy. Moreover, the crucibles herein can be heated rapidly without cracking during any of the melting, pouring, casting and cooling stages of the vacuum induction melting cycle.

The net result of this improved crucible performance is that the crucible is more resistant to thermal stresses and the TiAl melted therein remains more pure and has improved fatigue life. As used herein, "pure" means that the alloy has an oxygen content of less than about 1200 ppm by weight, and includes less than about 500 ppm by weight of yttrium or silicon contaminates generated by the crucible during the melting process. Due to this improved purity, components made from the TiAl exhibit less cracking and fewer imperfections than those made from TiAl using current methods.

This written description uses examples to disclose the invention, including the best mode, and also to enable any person skilled in the art to make and use the invention. The patentable scope of the invention is defined by the claims, and may include other examples that occur to those skilled in the art. Such other examples are intended to be within the scope of the claims if they have structural elements that do not differ from the literal language of the claims, or if they include equivalent structural elements with insubstantial differences from the literal language of the claims.

65 What is claimed is:

1. A method for making a reinforced refractory crucible for melting titanium alloys, the crucible having at least one side

region prone to hoop stresses and at least two regions that are separated by the side region and are prone to bending stresses, the method comprising:

forming a crucible mold on a form by:

applying a facecoat to the form;

applying at least one reinforcing element to at least a portion of the crucible mold defined by the facecoat layer, the backing layer, or a combination thereof, the at least one reinforcing element comprising a configuration selected from the group consisting of a continuous fiber, a tape, a mesh, and combinations thereof; wherein the step of applying the at least one reinforcing element comprises applying a first reinforcing element to a first portion of the crucible mold that corresponds to the side region of the crucible and applying a second reinforcing element to a second portion of the crucible mold that corresponds to at least one of the two regions of the crucible that are separated by the side region, the first reinforcing element comprises a continuous fiber that is wrapped around the first portion of the crucible mold, and the second reinforcing element comprises a mesh that is wrapped around the second portion of the crucible mold;

firing the crucible mold.

2. The method of claim 1 comprising applying a stucco layer to each of the at least one facecoat layer and the at least one backing layer.

3. The method of claim 2 comprising applying the at least one reinforcing element to at least a portion of the facecoat layer, the backing layer, the stucco layer, or combination thereof.

4. The method of claim 3 comprising applying the at least one reinforcing element to the entire facecoat layer, backing layer, stucco layer, or combination thereof.

5. The method of claim 1 wherein the at least one reinforcing element comprises at least one ceramic composition selected from the group consisting of yttria, alumina, sapphire, yttrium aluminum garnet, silicon carbide, silicon, aluminum oxynitride, mullite, zirconia, zircon, zircar, and combinations thereof.

6. The method of claim 1 wherein the at least one reinforcing element comprises at least one metallic composition selected from the group consisting of tungsten, tantalum, molybdenum, niobium, rhenium, alloys thereof, and combinations thereof.

7. The method of claim 1 wherein:

the facecoat has at least one facecoat layer comprising an oxide powder in a colloidal suspension, the oxide powder is selected from the group consisting of scandium oxide, yttrium oxide, hafnium oxide, a lanthanide series oxide, and combinations thereof, and the colloidal suspension is selected from the group consisting of colloidal silica, colloidal yttria, colloidal alumina, colloidal calcium oxide, colloidal magnesium oxide, colloidal lanthanide series oxides, and mixtures thereof; and the at least one reinforcing element comprises at least one composition selected from the group consisting of ceramic compositions, metallic compositions, and combinations thereof.

8. The method of claim 1 comprising applying the first and second reinforcing elements in a manner selected from the group consisting of an adjacent orientation, a stacked orientation, or combinations thereof.

9. The method of claim 8 comprising applying more than one of the first or second reinforcing element to the first or second portions, respectively, of the crucible mold.

10. A method for making a reinforced refractory crucible for melting titanium alloys, the crucible having at least one side region prone to hoop stresses and base and pour lip regions that are separated by the side region and are prone to bending stresses, the method comprising:

providing a form;

applying a facecoat to the form;

applying a backing about the facecoat, the backing having at least one backing layer;

applying at least one reinforcing element to at least a portion of the facecoat layer, the backing layer, or a combination thereof, the facecoat, the backing layer and the at least one reinforcing element defining a crucible mold; removing the form from the crucible mold;

applying a colloidal topcoat to the crucible mold; and firing the crucible mold;

wherein the at least one reinforcing element comprises a configuration selected from the group consisting of a continuous fiber, a tape, a mesh, and combinations thereof and the step of applying the at least one reinforcing element comprises applying a first reinforcing element to a first portion of the crucible mold that corresponds to the side region of the crucible and applying second reinforcing elements to second portions of the crucible mold that correspond to the base and pour lip regions of the crucible, the first reinforcing element comprises a continuous fiber that is wrapped around the first portion of the crucible mold, and the second reinforcing elements comprise meshes that are wrapped around the second portions of the crucible mold.

11. The method of claim 10 wherein the facecoat has at least one facecoat layer comprising an oxide powder in a colloidal suspension, the oxide powder is selected from the group consisting of scandium oxide, yttrium oxide, hafnium oxide, a lanthanide series oxide, and combinations thereof, and the colloidal suspension is selected from the group consisting of colloidal silica, colloidal yttria, colloidal alumina, colloidal calcium oxide, colloidal magnesium oxide, colloidal lanthanide series oxides, and mixtures thereof.

12. The method of claim 10 wherein the at least one reinforcing element comprises a composition selected from the group consisting of ceramic compositions, metallic compositions, and combinations thereof.

13. The method of claim 10 comprising:

applying a stucco layer to each of the at least one facecoat layer and the at least one backing layer; and

applying the first and second reinforcing elements in a manner selected from the group consisting of an adjacent orientation, a stacked orientation, or a combination thereof.

14. The method of claim 13 comprising applying the at least one reinforcing element to at least a portion of more than one of the facecoat layer, the backing layer, the stucco layer, or combinations thereof.

15. The method of claim 13 comprising applying the at least one reinforcing element to the entire facecoat layer, backing layer, stucco layer, or combination thereof.

16. A method for making a reinforced refractory crucible for melting titanium alloys, the crucible having at least one side region prone to hoop stresses and base and pour lip regions that are separated by the side region and are prone to bending stresses, the method comprising:

providing a form;

applying a facecoat to the form, the facecoat having at least one facecoat layer comprising an oxide powder in a colloidal suspension, the oxide powder selected from the group consisting of scandium oxide, yttrium oxide,

**11**

hafnium oxide, a lanthanide series oxide, and combinations thereof, and the colloidal suspension selected from the group consisting of colloidal silica, colloidal yttria, colloidal alumina, colloidal calcium oxide, colloidal magnesium oxide, colloidal lanthanide series oxides, and mixtures thereof;

applying a backing about the facecoat to produce a crucible mold, the backing having at least one backing layer;

applying a stucco layer to each of the at least one facecoat layer and the at least one backing layer;

applying at least one reinforcing element to at least a portion of the facecoat layer, the backing layer, the stucco layer, or a combination thereof wherein the at least one reinforcing element comprises a composition selected from the group consisting of ceramic compositions, metallic compositions, and combinations thereof;

removing the form from the crucible mold;

applying a colloidal topcoat to the crucible mold; and

subjecting the crucible mold to a first firing at a temperature of about 800° C. to about 1400° C. followed by a second firing at a temperature of about 1400° C. to about 1800° C. to produce the reinforced crucible for melting titanium alloys;

wherein the at least one reinforcing element comprises a configuration selected from the group consisting of a

10

15

20

**12**

continuous fiber, a tape, a mesh, a chopped fiber, and combinations thereof and wherein the at least one reinforcing element is tailored to support particular stresses present in the side, base and pour lip regions of the crucible by applying a first reinforcing element of the at least one reinforcing element to a first portion of the crucible mold that corresponds to the side region of the crucible and applying second reinforcing elements of the at least one reinforcing element to second portions of the crucible mold that correspond to the base and pour lip regions of the crucible, the first reinforcing element comprises a continuous fiber that is wrapped around the first portion of the crucible mold, and the second reinforcing elements comprise meshes that are wrapped around the second portions of the crucible mold.

**17.** The method of claim **16** comprising applying the at least one reinforcing element to the entire facecoat layer, backing layer, stucco layer, or a combination thereof.

**18.** The method of claim **16** comprising applying the first and second reinforcing elements in a manner selected from the group consisting of an adjacent orientation, a stacked orientation, or a combination thereof.

\* \* \* \* \*